

April 23, 1935.

J. A. ANDERSON

**1,998,648**

## DEWAXING LUBRICATING OILS

Filed July 9, 1932

3 Sheets-Sheet 1

Fig. 1



**INVENTOR**

INVENTOR  
*John A. Anderson*  
BY *Donald E. Payne*  
ATTORNEY

April 23, 1935.

J. A. ANDERSON

1,998,648

DEWAXING LUBRICATING OILS

Filed July 9, 1932

3 Sheets-Sheet 2



Fig. 2

INVENTOR  
John A. Anderson  
BY  
Donald E. Payne  
ATTORNEY

April 23, 1935.

J. A. ANDERSON

1,998,648

## DEWAXING LUBRICATING OILS

Filed July 9, 1932

3 Sheets-Sheet 3



Fig. 4.



## Modified wax crystals



Fig. 6.

## Modified wax crystals

## INVENTOR

INVENTOR  
John A. Anderson  
BY Donald E. Payne  
ATTORNEY

## UNITED STATES PATENT OFFICE

1,998,648

## DEWAXING LUBRICATING OILS

John A. Anderson, Chicago, Ill., assignor to  
 Standard Oil Company, Chicago, Ill., a corpora-  
 tion of Indiana

Application July 9, 1932, Serial No. 621,692

6 Claims. (Cl. 196—19)

This invention relates to the separation of wax from mineral oils and pertains more specifically to a method of crystallizing wax in a particular manner so that it may be readily separated from oil by cold settling or by centrifuge.

Most petroleum oils, particularly paraffin and mixed base oils, contain substantial quantities of paraffin wax which accumulate in lubricating oil fractions obtained by distillation. Mid-Continent lubricating distillates may contain 10% of paraffin wax; Salt Creek distillates as much as 20% wax. For most lubricating purposes, it is necessary to remove this wax so that the oil will not solidify at low temperatures. A very small amount of wax will greatly increase the pour point or the temperature at which the oil congeals. The object of my invention is to remove all of the waxy bodies from lubricating oil which are responsible for unduly high pour points.

Heretofore, it has been the custom to dilute oils with naphtha or other light hydrocarbons, to chill the diluted oil, to crystallize out the wax and to mechanically separate the wax by filtration, centrifuging or settling. Filtration is expensive, and is difficult because of the tendency to clog the filters and because of the low temperatures at which the separation must be effected. Cold settling is the simplest method of wax separation, but it is open to the objection that many waxes will not settle at all and many other waxes will not settle sufficiently to make this process commercially feasible. Paraffin wax crystallizes in the form of plates or needles which are rather irregular in outline and which interlock or interlace and set up a skeleton framework throughout the entire body of the oil, to all intents and purposes causing the body of oil to solidify. In many oils the amount or nature of the wax is such that that the oil is not solid, but even in these cases the interlacing of the wax crystals causes entrainment of so much oil that the oil and wax cannot be readily separated by cold settling. If such chilled diluted waxy oil is settled in a tank 100 units deep, the wax crystals may only settle a few units from the top; if they settle 10 units, it is said that the oil is settled to 90% bottoms. The object of my invention is to provide a method and means for separating waxy oil by a cold settling process wherein the diluted oil and wax mixture

50 may be settled to about 10% or 15% bottoms. In other words, I want to minimize the amount of oil which is entrained by wax and which is either carried down with it or which prevents it from settling.

55 A further object of my invention is to provide a

process of dewaxing which will require a minimum initial cost, a minimum amount of space and a minimum operating expense, which will at the same time give maximum yield of wax-free low cold test oil. Other objects will be apparent as the detailed description of my invention proceeds.

In practicing my invention I utilize certain condensation products to bring about the crystallization of wax in a readily settleable form. I add the condensation product before the dewaxing step and make use of it specifically to cause the crystallization of wax in a form which can be readily settled or centrifuged. My theory is that these condensation products cause wax to solidify in compact particles instead of in elongated plates or crystals and I reason from this hypothesis that diluted oil can be chilled and settled to low bottoms because the interlacing of wax crystals will be prevented. Microscopic examinations confirm this theory and actual tests have demonstrated that diluted oil which is 100% solid at  $-10^{\circ}$  F. can be settled to 8% to 15% bottoms by these condensation products. I have further discovered that the clear supernatant oil is characterized by a very low pour point, that the settling rate is much higher than can be otherwise obtained, and that markedly increased yields may be obtained.

My invention will be more clearly understood from the following detailed description and from the accompanying drawings which form a part of this specification and in which:

Figure 1 represents diagrammatically an elevation of my improved batch settler.

Figure 2 represents diagrammatically an elevation of my continuous settler.

Figure 3 represents diagrammatically an elevation of a centrifuge system, and

Figure 4 illustrates the microscopic appearance of wax crystal structure in the absence of a condensation product;

Figure 5 illustrates the microscopic appearance of wax crystals formed in the presence of a condensation product; and

Figure 6 illustrates the microscopic appearance of another form of wax crystal structure in the presence of a condensation product.

My invention will be described in connection with the dewaxing of Mid-Continent treated distillate oil having a viscosity of about 74 seconds 50 Saybolt at  $210^{\circ}$  F. I do not limit myself, however, to any particular type of wax-bearing oil,—the invention is applicable to oils with viscosities of 90 seconds at  $210^{\circ}$  F. and 100 seconds at 100° F., all distillates, untreated as well as treated,

5

10

15

20

25

30

35

40

45

50

55

light as well as heavy, Pennsylvania, Coastal, etc. as well as Mid-Continent, etc.,—any oil containing difficultly settleable wax.

My condensation products may be described as 5 a resinous material formed by condensation of halogenated hydrocarbons, with aromatic compounds in the presence of a catalyst such as aluminum chloride, the condensation preferably being effected in a suitable solvent. As a halogenated hydrocarbon I prefer to use chlorinated 10 paraffin wax having a melting point of about 130° F. before chlorination and being chlorinated to about 15%. I may use other hydrocarbons, however, such as petrolatum, Montan wax, viscous 15 oils, etc., and I may vary the amount of chlorination over a relatively wide range, although I prefer to use a hydrocarbon with about 10% to 20% of added chlorine. The aromatic compound is 20 preferably naphthalene or diphenyl, although other compounds, such as benzene and toluene, may also be used. I prefer to effect the condensation 25 in the presence of a chlorinated liquid, such as carbon tetrachloride, chloroform, tetrachloroethane, etc., although other liquid, such as naphtha, may be used if desired. Aluminum 30 chloride or its equivalent has been found to be the best catalyst.

One specific example of my condensation product may be made up as follows:

30 About 15 parts by weight of aluminum chloride is slowly added with stirring to a solution of 100 parts by weight of chlorinated wax (130° F. melting point with 15% chlorine) and 15 parts of naphthalene in enough carbon tetrachloride to 35 maintain all of the ingredients in solution. The temperature of addition and subsequent stirring is about 130° to about 140° F., and the mixture is stirred for a period of 8 or 10 hours (or until the reaction is complete). The sludge is then allowed to settle and the upper liquid is withdrawn 40 and distilled to remove the diluent and the unreacted hydrocarbon and perhaps a part of the hydrocarbon material as distillates. The remaining heavy oil or resin is my condensation 45 product.

As another example, about 25 parts of aluminum chloride may be slowly added to 25 parts of naphthalene and 100 parts of chlorinated wax in a chloroform solution. Here again the 50 optimum temperature is about 130° to 140° F. The reaction is usually complete in from one to ten hours.

As above stated, I may use a wide variation of chlorinated or halogenated waxes or hydrocarbons and I may vary the aromatic compound and the conditions of condensation throughout a relatively wide range. The expression "condensation product" as used in the following specification and claims is hereby defined to include that 55 class of substances prepared in the manner hereinabove set forth.

Referring to Figure 1, the treated (or untreated) waxy lubricating oil distillate is introduced by pipe 10 and mixed with about 0.1% of 60 my condensation product, which is transferred from storage tank 11 through pipe 12 by means of pump 13. The waxy oil with the condensation product mixed therewith is introduced by pipe 14 to mixer 15 where it is mixed with a diluent 65 such as propane from storage tank 16 and pipe 17, about five parts of propane being added to one part of waxy oil. This mixture is then selectively introduced by pipes 18 and 19 or 20 into cooling or chill chambers 21 and 22. These 70 chambers may be refrigerated in any suitable

manner by the use of brine coils or by direct expansion of ammonia. I prefer, however, to refrigerate by vaporization of part of the diluent, propane vapors being withdrawn through reducing valves 23 and pipes 24 to low pressure gas main 25. Propane from main 25 is compressed by pump 26, condensed in coils 27, cooled in chamber 28 and finally returned to storage tank 16. 5

The diluted oil-wax mixture may be chilled at the rate of about 3° F. per minute. The original 10 mixture may be at a temperature of about 80° to 100° F. and the mixture in the chill chambers is reduced to a temperature of about -40° F. This cold slurry is then selectively introduced by pipes 29 or 30 and 31 or 32 to settling tanks 33 or 34. 15 It should be understood that by using a plurality of these tanks one tank may be filled while another is being cooled, etc. Further cooling may be effected in settling tanks by removing of propane vapors through reducing valves 35 and 20 36 to low pressure gas line 25. In fact, I may use the settling tanks to effect the entire chilling by passing the diluted waxy oil mixture directly from mixer 15 through pipes 18, 37, and 31 or 32. If additional propane is required as diluent and/or 25 refrigeration in chill chambers it may be introduced through line 38.

The rapidity with which the wax crystals settle out in settling tanks 33 and 34 will depend to a 30 large extent upon the nature of the waxy oil, the nature of the diluent and the amount and quality of the condensation product. If the Mid-Continent stock above described is chilled in the absence of the pour condensation product, the wax will crystallize in the form of interlacing 35 needles 39, as shown in Figure 4. By using condensation product the wax assumes the form of tiny slightly star-shaped aggregate 40 or tiny rounded particles 41 (see Figure 4), which settle rapidly and to very low bottoms. In one series 40 of experiments, for instance, it was shown that without the use of condensation products the wax did not settle at all—it gave 100% bottoms; when 0.3% of the condensation product was added, the wax settled to 17% bottoms, and this settling 45 from propane required less than an hour.

The clear oil may be decanted from either settling tank through pipe 42 through outlets 43, 44, 45, 46 and 47. Pet cocks (not shown) are provided adjacent these outlets for sampling the 50 oil before it is decanted. By having a plurality of these tanks, one of them may be settling while another is being emptied and furthermore, the oil may be decanted from the upper part of the tank while the wax is settling still further in the 55 lower part. When the clear wax-free oil has been decanted, I remove the remaining wax slurry from the base of the settlers through pipes 43 and 44, usually this wax is in the form of a slurry so that it may be readily handled as a liquid, but if 60 desired I may melt it by means of steam coils 45 or by other suitable heating means. The wax may be washed several times with propane or reprecipitated therefrom, the propane being recovered by means of suitable stripping stills (not 65 shown).

The cold wax-free diluted oil may be collected in a suitable sump or receiver and then passed by means of pump 46 and pipe 47 to exchanger 28 wherein it absorbs the heat from liquefied propane. The warm mixture is then passed by pipe 48 to stripping stills 49 equipped with steam heater coil 50, the finished oil being withdrawn through pipe 51 and propane being returned to the low pressure gas line through pipe 52. 75

In Figure 2 I have shown a similar embodiment except that instead of using a plurality of batch settling tanks I use a large continuous settler 53 which may be in the form of a hopper bottomed cylinder or a large horizontal tank. In this case, the wax slurry is continuously removed from the base of the settler by means of screw conveyor 54 and the clear oil is directly introduced by pipe 55 to the stripper 49. In all other respects this modification is the same as that described in connection with Figure 1.

Referring to Figure 3, it will be observed that the slurry from the chill chambers is introduced into the centrifuge 56 instead of into its cold settling tanks. This centrifuge may be of the type commonly used in the oil industry and may be driven by motor 57. The wax may be delivered by pipe 58 to collector 59 and it may be transferred therefrom through pipe 60 by pump 61 to stripping still 62, which is heated by steam coil 63, the wax being withdrawn through pipe 64 to suitable storage tank and the propane being returned through pipe 55 to low pressure gas line. The diluted wax-free oil is withdrawn from centrifuge 25 through pipe 66 to collector 67, from which it is pumped through pipe 68 by pump 69 to stripping still 49 as hereinabove described.

When the Mid-Continent distillate was cold settled with four volumes of propane without the use of a condensation product and the chilled mixture was allowed to stand for over six hours, the yield of finished oil was 63% of the weight of the original charge, and the pour point of the finished oil was about +3° F. When the condensation product of chlorinated paraffin wax and naphthalene was added prior to the settling, the settling rate was markedly increased, the yield was about 10% higher and the pour point of the finished oil was below 0° F.

In another series of tests using filter naphtha as a diluent in the ratio of three parts waxy oil to seven parts naphtha and using about 0.1 to 0.3% of the condensation product referred to above, I obtained 17% bottoms from a diluted oil-wax mixture which was absolutely solid under the same conditions without the small amount of condensation products.

Generally speaking, the effects of the condensation products in increasing settling rates and decreasing the bottoms, is more useful with larger amounts of diluent and with lighter diluents (higher A. P. I. gravity or lower specific gravity).

The microscopic examination of wax solidified from overhead cuts with and without the use of condensation products supports my theory of how and why I obtain my improved results. Heretofore this wax crystallized out in the form of interlacing plates or needles throughout the entire mass of the liquid, thereby entraining the oil and supporting other wax crystals. It is obvious that in such a system settling is impossible. The condensation products prevent this type of crystallization and cause the formation of small aggregates of needles or tiny rounded particles which have no tendency to interlock and which may be readily settled or centrifuged.

Instead of using propane as a diluent I may use naphtha, normally gaseous light hydrocarbon diluents, such as butane, iso-butane, propylene, butylene, etc., antisolvents such as acetone, methyl formate, nitrobenzene, etc. or mixtures thereof with miscibility agents, such as benzol and toluol. In other words, the invention is of greatest value in light diluents such as propane, but it is not limited thereto.

The apparatus will, of course, be suitably insulated and provided with valves, pumps, collector tanks, etc. All of these engineering details are commonly known in the art. They form no part of the present invention and they will therefore not be described in detail.

The amount of condensation products used may vary considerably. About 0.1 to 0.3% of the concentrated resins gives excellent results, but much larger quantities can be used if desired.

While I have described my invention in detail and have set forth a theory of operation, it should be understood that I do not limit myself to either the details nor the theory except as defined by the following claims, which should be construed as broadly as the prior art will permit.

I claim:

1. The method of separating wax from wax-bearing mineral oil which comprises adding to said oil a synthetic product formed by the addition of aluminum chloride to a mixture of naphthalene and chlorinated wax, diluting said oil with a diluent, chilling the diluted mixture to effect solidification of the wax, mechanically removing the wax from the diluted oil, and removing the diluent from the wax-free oil.

2. The method of separating wax from a wax-bearing animal oil which comprises admixing with a waxy oil and a diluent a small amount of a synthetic product formed by the reaction of naphthalene with chlorinated wax by the addition of aluminum chloride, chilling the mixture to effect solidification of the wax in the form of small aggregates, separating the solidified wax from the diluted oil, and separating the diluent from the wax-free oil.

3. The method of accelerating the rate of settling and increasing the wax-free oil yield of a cold settling process which comprises diluting a wax-containing oil with a diluent, adding to said diluted oil a small amount of a condensation product formed by the reaction of naphthalene with a chlorinated wax by the addition of aluminum chloride thereto, chilling said diluted oil-wax mixture in the presence of said condensation product to cause the solidification of wax without the formation of interlacing crystals, and allowing said cold mixture to settle.

4. The method of claim 1 wherein about .1% to about .3% of the synthetic product is added to the wax-bearing oil, based on the weight of the wax-bearing oil.

5. The method of claim 1 wherein the synthetic product is prepared by condensing the chlorinated wax with the naphthalene, both dissolved in a halogenated liquid, the aluminum chloride being added to said ingredients.

6. The method of separating wax from a wax-bearing mineral oil, which comprises diluting said oil with a light diluent for reducing its viscosity, adding to said oil a small amount of a crystallization inhibitor formed by reacting a halogenated hydrocarbon with an aromatic compound by slowly adding aluminum chloride to a molten mixture of said halogenated hydrocarbon and aromatic compound at a temperature of about 130° to 140° F., cooling the diluted oil containing the crystallization inhibitor to effect solidification of the wax in the form of small aggregates, separating the wax from the diluted oil by utilizing their difference in specific gravity, and separating the diluent from the wax-free oil.

JOHN A. ANDERSON.